

# United States Patent Office

2,796,423

Patented June 18, 1957

1

2,796,423

## FORMALS OF LUBRICATING GRADE

Delmer L. Cottle, Highland Park, and David W. Young, Westfield, N. J., assignors to Esso Research and Engineering Company, a corporation of Delaware

No Drawing. Application December 1, 1952,  
Serial No. 323,503

6 Claims. (Cl. 260—410.9)

This invention relates to synthetic lubricating compositions. Particularly the invention relates to synthetic lubricating compositions having outstanding lubricating properties at both high and low temperatures and which have the advantage of leaving substantially no combustion chamber deposits in the cylinders of reciprocating engines. More particularly the invention relates to new and improved synthetic lubricating oils which comprise the formals of organic compounds having at least one free hydroxyl group which is alcoholic in nature.

In recent efforts to obtain superior lubricating compositions which have unusual and specific properties, there have been developed entirely new synthetic materials with lubricating properties. In general these new synthetic lubricants are characterized by viscosity properties that are outstanding at both low and high temperatures, especially when compared to mineral oils. These outstanding low and high temperature properties are especially desirable for use in equipment designed to operate over a great temperature differential, such as jet engines or turbines for aircraft use, internal combustion reciprocating engines for aircraft and the like. It has been found that mineral lubricating oils have generally undesirable limitations for the lubricating of these engines, particularly in respect of their high and low temperature viscosity characteristics.

It has also been found that synthetic lubricants may be desirable for the lubrication of standard automotive engines. In addition to the versatility of their viscosity-temperature relationships, some types of the synthetic lubricants investigated have another advantage in that their use has been found to result in very low rates of combustion chamber deposit formation, particularly when they are used for long periods of time. Low rates of formation of combustion chamber deposits result in a more efficient utilization of fuel, less increase in the octane requirement of an engine, less pre-ignition tendency, and a general overall improvement in engine operation. These lubricants may also serve to reduce or remove combustion chamber deposits from an engine already containing such deposits.

The present invention relates to a new type of synthetic lubricating composition which comprises the formals of a wide range of organic compounds which contain at least one free hydroxyl group which is alcoholic in nature. The term formal is meant to cover compounds containing the  $-\text{O}-\text{CH}_2-\text{O}-$  group.

It has been generally accepted by the art that acetals in general are not of sufficient stability to serve as lubricating compositions. It has now been found, however, and forms the object of this invention, that the formals of organic hydroxy compounds, wherein two molecules, each containing one or more free hydroxyl groups which have an alcoholic nature are joined through a methylene group ( $-\text{CH}_2-$ ) have excellent stability and have viscosity properties that make them outstanding lubricating compositions. In the formation of these compounds, the methylene group replaces a hydrogen

2

of an alcoholic hydroxyl group on each of two molecules and links them in one molecule.

A generic formula for the lubricating compositions of this invention may be written as follows:



In the formula A and B represent radicals which are the organic hydroxy compounds less the reacting hydrogen atoms. These radicals may be alike or different and may contain from 1 to 60 carbon atoms. A and B are selected such that the total number of carbon atoms in the average formal molecule produced by the reaction is between about 20 and 130, with compounds containing from about 25 to 100 carbon atoms being preferred. The organic hydroxyl compounds which serve as a source for the radicals A and B will be defined more in detail below.

For use in reciprocating engines, particularly as a lubricant for automotive engines, a lubricating composition must meet several requirements. In order to form an effective lubricating film and to maintain that film at low and high temperatures it must have certain viscosity characteristics. At low temperatures the lubricant must be sufficiently labile to flow through the circulatory system of the equipment and allow movement of lubricated surfaces without an undue power requirement. A lubricant having an ASTM pour point below about  $+35^{\circ}\text{ F.}$  has sufficient low temperature lability to make it satisfactory in these respects for general use. At high temperatures a lubricant must have sufficient "body" or "thickness" to furnish and maintain a satisfactory lubricating film. It has been found that a lubricant that is satisfactory in this respect will have a viscosity at  $210^{\circ}\text{ F.}$  of between about 2 to 60 centistokes of about 30 to 280 Saybolt seconds, Universal. To prevent undue lubricant loss due to volatility and general molecular disintegration, and to insure against explosion hazards at higher temperatures sometimes encountered, a lubricating composition should have a flash point in excess of about  $300^{\circ}\text{ F.}$  These requisites are inherent in the term "lubricating compositions," as used in this specification, and the formals of this invention are limited to those within these operable ranges. The preferred materials, as contemplated herein and as described in the preferred embodiment hereof, will have an ASTM pour point below about  $-15^{\circ}\text{ F.}$ , a flash point above about  $375^{\circ}\text{ F.}$ , and will have a viscosity within the range of 2.6 to 13 centistokes or 35 to 170 Saybolt seconds, Universal, at  $210^{\circ}\text{ F.}$

In general it has been found that the above listed properties are a function both of molecular structure and of molecular weight. This fact makes it possible, within certain limits, to prepare compositions having similar low and high temperature properties in a variety of ways and also enables the manufacturer to "tailor" a composition to fit a certain set of specifications within rather general limits. The large number of organic materials containing alcoholic hydroxyl groups available for preparing the compositions of this invention makes it possible to prepare a wide range of lubricants.

As was stated above the formals of the instant invention are prepared from organic hydroxy compounds containing at least one free hydroxyl group which is alcoholic in nature. These organic hydroxy compounds may contain as few as 1 carbon atom or as many as 60 carbon atoms. It is essential, however, that the total number of carbon atoms in the average formal molecule be between about 20 to about 130, with from 25 to 100 total carbon atoms being especially preferred. Those formals containing fewer than about 20 carbon atoms have been found to be lacking in desirable high temperature viscosity characteristics and those having more than about

130 are usually too viscous at low temperatures. The materials used to prepare these formals, that is, organic hydroxy compounds containing at least one free hydroxyl group which is alcoholic in character, may be selected from the following partial list. Others may of course be used.

**I. Unsubstituted alcohols**

**A. Monohydric**

1. Aliphatic
  - (a) Methyl alcohol
  - (b) Ethyl alcohol
  - (c) Propyl alcohol
  - (d) Isopropyl alcohol
  - (e) n-Butyl alcohol
  - (f) Iso-butyl alcohol
  - (g) Sec.-butyl alcohol
  - (h) Tert.-butyl alcohol
  - (i) n-Amyl alcohol
  - (j) Iso-amyl alcohol
  - (k) n-Hexyl alcohol
  - (l) Iso-hexyl alcohol
  - (m) 2-ethyl-1-butanol
  - (n) 2-ethyl-1-hexanol
  - (o) Octyl alcohol
  - (p) Iso-octyl alcohol
  - (q) 2-octanol
  - (r) Iso-nonyl alcohol
  - (s) Decyl alcohol
  - (t) Lauryl alcohol
  - (u) Tetradearyl alcohol
  - (v) Pentadearyl alcohol
  - (w) Octadearyl alcohol
  - (x) Allyl alcohol
  - (y) Crotyl alcohol
  - (z) Oleyl alcohol
  - (aa) The terpineols
  - (bb) C<sub>8</sub> to C<sub>20</sub> oxo alcohols
  - (cc) Alcohols derived from the "Synol" process
  - (dd) Alcohols derived from the oxidation of petroleum fractions
  - (ee) Alcohols derived from Guerbet's reaction
  - (ff) Alcohols derived from the hydration of olefins
  - (gg) Alcohols derived via the "Oxyl" synthesis
  - (hh) Mixtures of the above

2. Aromatic

- (a) Benzyl alcohol
- (b) Phenethyl alcohol
- (c) 3-phenyl-1-propanol
- (d)  $\alpha$ -Naphthyl carbinol
- (e) Cinnamyl alcohol
- (f) Diphenyl carbinol
- (g) Furfuryl alcohol
- (h) Cumaric alcohol
- (i) Vanillyl alcohol
- (j) Piperonyl alcohol

**B. Polyhydric**

1. Glycols

- (a) Ethylene glycol
- (b) 1,2-propanediol
- (c) 1,3-propanediol
- (d) 1,3-butanediol
- (e) 1,4-butanediol
- (f) 1,5-pentanediol
- (g) The various polyalkylene glycols, e. g.
  1. Polyethylene glycols
    - (a) Diethylene glycol
    - (b) Triethylene glycol
    - (c) Tetraethylene glycol
  2. Polypropylene glycols
    - (a) Dipropylene glycols
    - (b) Tripropylene glycol

(h) 1,2-cyclohexanediol

(i) Decanediol-1,10

2. Other polyhydric alcohols

- (a) Glycerol
- (b) 2-hydroxymethyl-2-methyl propanediol-1,3
- (c) Pentaerythritol
- (d) Sorbitol
- (e) Dipentaerythritol
- (f) Dulcitol
- (g) Trimethylol propane
- (h) Tetramethylol cyclohexanol
- (i) Benzotrimethylol

**II. Substituted alcohols**

**A. Monohydric**

1. Aliphatic

- (a) Halogenated alcohols
  1. Ethylene chlorohydrin
  2. Trifluoro ethanol
  3. Propylene chlorohydrin
  4. The various chloro-substituted mono-ethers of polyalkylene glycols
- (b) Ethanolamine
- (c) 2-amino propanol
- (d) 2-nitroethanol
- (e) 2-nitropropanol
- (f) 2-nitrobutanol
- (g) The various glycol monoesters, e. g.
  1. Ethylene glycol monoacetate
  2. Propylene glycol monobutyrate
  3. Butylene glycol monolaurate
  4. Polyethylene glycol monoesters
  5. Polypropylene glycol monoesters
  6. Polybutylene glycol monoesters
- (h) The various glycol monoethers, e. g.
  1. Ethylene glycol mono-methyl ether
  2. Propylene glycol mono-butyl ether
  3. Butylene glycol mono-lauryl ether

4. Polyethylene glycol mono-ethers
5. Polypropylene glycol mono-ethers
6. Polybutylene glycol mono-ethers
7. Polytrimethylene glycol mono-ethers
- (i) The various glycol mono-formals, e. g. the mixed formals of glycols and alcohols
- (j) Hydroxy alkyl cyanides
1. Ethylene cyanohydrin
2.  $\alpha$ -Hydroxy isobutyronitrile
- (k) Ethanol morpholine

2. Aromatic

- (a) p-Methoxy benzyl alcohol
- (b) The various chlorobenzyl alcohols
- (c) The various nitrobenzyl alcohols
- (d) 2-anilino ethanol

B. Polyhydric

1. Glycols

- (a) Halogenated glycols, e. g.
  1. 3-chloro-1,2-propanediol
  2. 2-chloro-1,3-propanediol

(b) Nitroglycols, e. g.

1. 2-nitro-1,3-propanediol
2. 2-nitro-2-methyl-propanediol-1,3
3. Trimethylol nitromethane

(c) Amino glycols

1. 2-amino-1,3-propanediol
2. 2-amino-2-methyl-1,3-propanediol
3. Diethanol amine
4. Trimethylol aminomethane

C. Other hydroxy compounds

1. Esters of hydroxy acids

- (a) The various lactate esters

- (b) The various glycolate esters

- (c) The various hydroxy stearate esters

2. Carbonyl substituted alcohols

- (a) Hydroxy ketones, e. g.
  1. Hydroxy acetone
  2. Hydroxy aldehydes, e. g.

1.  $\alpha$ -Hydroxy adipaldehyde
2.  $\beta$ -Hydroxy propionaldehyde

Particularly desirable organic hydroxyl compounds for use in this invention are those highly branched chain aliphatic alcohols prepared by the "Oxo" synthesis. The "Oxo" synthesis may be described as being the catalytic reaction of an olefin with carbon monoxide and hydrogen. The reaction occurs at temperatures in the order of 300°-400° F., at pressures in the range of about 1000 to 3000 p. s. i., in the presence of a suitable catalyst, ordinarily a heavy metal carbonyl such as cobalt carbonyl. The resulting aldehyde is subsequently hydrogenated to a primary alcohol. This process is described in U. S. Patent No. 2,327,066 issued to Roelen in 1943.

In general the oxygenated group in a product from an olefin by the Oxo process is thought of as becoming attached to an unsaturated carbon which holds at least one hydrogen atom. In those cases where the carbon monoxide attacks a "saturated" carbon atom, it must be assumed either that that carbon has become unsaturated prior to reaction by a shift of a hydrogen atom or that the attack is directly on a carbon atom that is truly saturated. For example, 2-butene has been reported to give 1-pentanol and 2-methylbutanol in equal quantities, a result that cannot be explained on the simple basis that oxonation takes place only on unsaturated carbons holding hydrogen. 2,3-dimethyl-2-butene also reacts giving only 3,4-dimethyl-1-pentanol; in this olefin no hydrogen is attached to the unsaturated carbon atoms and the attack of carbon monoxide must either be on a "rearranged" olefin or on a saturated carbon atom.

It has been found that particularly desirable alcohols for the formation of the formals of this invention can be prepared by the application of the Oxo synthesis to polymers and copolymers of C<sub>3</sub> and C<sub>4</sub> monoolefins. These monoolefins are readily available in petroleum refinery streams, and processes for their conversion to liquid copolymers have been worked out by the art. One such process, known as U. O. P. polymerization, consists of passing the olefin-containing stream in liquid phase in contact with an acid catalyst comprising phosphoric acid impregnated on kieselguhr. Other acidic catalysts, such as phosphoric acid or copper phosphate impregnated on silica gel, sulfuric acid, Friedel-Crafts catalysts, activated clays, silica-alumina, copper pyrophosphate, etc. may be used. Suitable conditions when employing phosphoric acid catalysts of the U. O. P. type are temperatures of 300° F. to 500° F., pressures from 250 to 5,000 p. s. i. and feed stocks comprising refinery streams containing propylene and mixed butylenes. Suitable feed stocks,

for example, may contain from 15 to 60 mol percent propylene, from 0.5 to 15 mol percent butylenes, and from 0.1 to 10 mol percent isobutylene, the remaining being saturated hydrocarbons. Other suitable feed stocks are the dimer and trimer of isobutylene.

The preferred Oxo alcohols employed in forming the formals of this invention are those having from 8 to 20 carbon atoms derived from olefin copolymers having from 7 to 19 carbon atoms. In preparing these Oxo alcohols the desired olefin fraction is segregated from the crude olefin polymer product by fractionation.

The following table, for example, shows the structure and percent composition of C<sub>8</sub> Oxo alcohols prepared from a C<sub>7</sub> olefin stream which had been fractionated from the products obtained by the phosphoric acid polymerization of refinery gas streams containing propylene and mixed n- and isobutylenes.

| Structure of C <sub>8</sub> Oxo Alcohols Prepared From C <sub>3</sub> -C <sub>4</sub> Copolymer Heptenes | Percent |
|----------------------------------------------------------------------------------------------------------|---------|
|                                                                                                          | 29      |
|                                                                                                          | 17      |
|                                                                                                          | 16      |
|                                                                                                          | 2.3     |
|                                                                                                          | 1.4     |
|                                                                                                          | 4.3     |
|                                                                                                          | 5.0     |
|                                                                                                          | 100.0   |
| $\alpha$ -alkyl-alkanols.....                                                                            |         |
| Others.....                                                                                              |         |

It will be noted that Oxo alcohols derived from the olefins produced by C<sub>3</sub>-C<sub>4</sub> polymerization are mostly methyl substituted.

The preparation of the formals of invention may be carried out as follows:

Formaldehyde in aqueous solution or any of the polymers of formaldehyde, such as paraformaldehyde, is refluxed with the desired organic material containing the hydroxyl group or groups. Acidic materials such as hydrochloric acid, sulfuric acid, sulfamic acid, p-toluenesulfonic acid, sodium acid sulfate, phosphoric acid, phosphoric acid deposited on a silica containing compound such as kieselguhr, ion exchange resins or any inorganic acidic substance may be used as a catalyst. Entrainning liquids such as hexane, heptane fractions, benzene and the like may be used in order to remove the water of reaction, although good yields are readily obtainable without a water entrainer.

These formals also may be made by acetal interchange wherein a formal such as methylal is heated with an alcohol to form a higher molecular weight formal. The methanol may be recovered, reconverted to methylal and recycled. Formals such as di-n-butyl formal may be used with an alcohol of higher boiling point than the n-butyl alcohol, the n-butyl alcohol that is formed being removed intermittently or continuously in order to increase the yield of the higher formal. The catalysts for this reaction also are acidic although other types of catalysts may be used.

The product may be water washed followed by an alkali wash and dried over some suitable drying agent, such as anhydrous potassium carbonate, or by distillation using a hydrocarbon as a water entrainer. Final distillation or stripping may be under reduced pressure if desired.

As was stated above, the synthetic lubricating oils of this invention comprise formals having the general formula:



wherein A and B are alike or different and are organic radicals derived from organic materials containing an alcoholic hydroxyl group. The radicals represented by A and B have from 1 to 60 carbon atoms each, and the total carbon atoms in the average molecule of the product number from 20 to 130 with 25 to 100 being a preferred range. Although any of the organic hydroxy containing materials listed hereinbefore may be used to prepare the formals of this invention, it has been found advantageous to utilize the radicals from alcohols and glycols, etc., and to build molecules having properties within the desired range by joining these hydroxyl containing materials through a formal linkage. Some possible combinations of these molecules are graphically depicted below.

For example, using compounds containing an alcoholic hydroxyl group and formaldehyde preferably with an acid catalyst and using well-known laboratory techniques the following molecules may be constructed:

- 17 Alcohol-formaldehyde-alcohol
- 25 Glycol-formaldehyde-alcohol
- 25 Glycol-formaldehyde-glycol
- 30 Glycol monoether-formaldehyde-alcohol
- 30 Glycol monoether-formaldehyde-glycol
- 35 Glycol monoether-formaldehyde-glycol monoether
- 35 Glycol monoester-formaldehyde-alcohol
- 35 Glycol monoester-formaldehyde-glycol
- 35 Glycol monoester-formaldehyde-glycol monoether
- 35 Glycol monoester-formaldehyde-glycol monoester

The acid used to prepare the glycol monoester may be selected from the following partial list:

|                  |                                               |
|------------------|-----------------------------------------------|
| Acetic           | Methoxy propionic                             |
| Propionic        | Ethoxyethoxyacetic                            |
| Butyric          | Mono-2-ethylhexyl adipate                     |
| 2-ethylbutyric   | Mono-C <sub>20</sub> Oxo acids including bot- |
| Caproic          | tom acids                                     |
| 2-ethyl hexanoic | Acids derived from petroleum                  |
| Caprylic         | fractions by oxidation                        |
| Pelargonic       | Acids derived from alcohols by                |
| Capric           | alkali fusion                                 |
| Lauric           | Naphthenic acids                              |
| Myristic         | Glycolic                                      |
| Oleic            |                                               |
| Stearic          |                                               |

To more specifically illustrate the concept of the instant invention the following examples are given. It is to be realized, of course, that these examples only illustrate the great number of possibilities that are covered by the inventive concept.

#### FORMALS OF SIMPLE ALCOHOLS

In all of the examples described below, unless otherwise specified, the product formed from the alcohol and formaldehyde was washed with alkaline solutions while hot and dried with anhydrous potassium carbonate, or by water entrainment, before being stripped or distilled at reduced pressure. Unless otherwise specified the alcohol and formaldehyde were reacted in stoichiometric amounts.

It is believed that the reaction proceeds according to the following equation:



Although it has been found that the reaction proceeds most favorably at the temperatures designated in the equation given above, these temperatures will depend upon the materials used, the catalyst, removal of water as formed, etc., and may vary from the range shown.

*Example 1*

The formal of  $C_{10}$  Oxo alcohol was prepared from paraformaldehyde and the alcohol at a final liquid temperature of  $198^{\circ}$  C. without a catalyst. The water was entrained with xylene and the residue boiling above a liquid temperature of  $185^{\circ}$  C. at 6 mm. was taken as product.

*Example 2*

The formal of  $C_{11}$  Oxo alcohol was prepared from paraformaldehyde and the alcohol by refluxing at a liquid temperature of  $112^{\circ}$  C. with 3.6 wt. percent of concentrated hydrochloric acid catalyst. The product distilled at  $147^{\circ}$ – $155^{\circ}$  C. at 3 mm.

*Example 3*

The mixed formal of  $C_{10}$  and  $C_{13}$  Oxo alcohols was prepared from an equimolar mixture of the alcohols and a stoichiometric amount of paraformaldehyde with 3.5 wt. percent concentrated hydrochloric acid catalyst. The product distilled at  $150^{\circ}$ – $174^{\circ}$  C. at 2 mm.

*Example 4*

The formal of  $C_{13}$  Oxo alcohol was prepared from the alcohol and an aqueous formaldehyde solution by refluxing with 3 wt. percent concentrated hydrochloric acid catalyst. The residue boiling above  $200^{\circ}$  C. liquid temperature at 7 mm. was taken as product.

*Example 5*

The formal of  $C_{13}$  Oxo alcohol was prepared from the alcohol and paraformaldehyde by refluxing with 3.1 wt. percent concentrated hydrochloric acid as the catalyst. The product distilled at  $160^{\circ}$ – $164^{\circ}$  C. at 1 mm.

*Example 6*

The formal of  $C_{13}$  Oxo alcohol was prepared from the alcohol and paraformaldehyde, entraining the water formed with benzene. The catalyst was 2.3 wt. percent concentrated sulfuric acid and the liquid temperature was  $162^{\circ}$  C.

*Example 7*

The formal of  $C_{13}$  Oxo alcohol was prepared from the alcohol and paraformaldehyde with 1 wt. percent benzene-sulfonic acid catalyst. The water was entrained with a commercial hexane fraction and the final liquid temperature was  $120^{\circ}$  C. The product distilled at  $163^{\circ}$ – $170^{\circ}$  C. at 7 mm.

*Example 8*

The formal of  $C_{13}$  Oxo alcohol was prepared similarly to that of Example 7. The catalyst was 1 wt. percent p-toluenesulfonic acid and the final liquid temperature was  $130^{\circ}$  C. The product distilled at  $163^{\circ}$ – $169^{\circ}$  C. at 7 mm.

*Example 9*

The formal of  $C_{13}$  Oxo alcohol was prepared from the alcohol and paraformaldehyde without a catalyst and with n-hexane as a water entrainer. The residue boiling above  $170^{\circ}$  C. at 7 mm. was taken as product.

*Example 10*

The formal of  $C_{13}$  Oxo alcohol was prepared from the alcohol and paraformaldehyde with 1 wt. percent sodium acid sulfate catalyst and n-hexane as the water entrainer. The product was filtered from the catalyst, was not washed, and distilled at  $165^{\circ}$ – $177^{\circ}$  C. at 5 mm.

*Example 11*

The formal of  $C_{13}$  alcohol was prepared as in Example 10 but was washed before distillation. It distilled at  $165^{\circ}$ – $181^{\circ}$  C. at 5 mm.

*Example 12*

The formal of  $C_{13}$  alcohol was prepared similarly to that in Example 10 except that the residue boiling above  $163^{\circ}$  C. at 4 mm. was taken as product.

*Example 13*

The formal of  $C_{13}$  alcohol was prepared from the alcohol and paraformaldehyde with 0.5 wt. percent sodium acid sulfate catalyst and a commercial heptane fraction as a water entrainer. Similar preparations were with 0.25 and 0.125 wt. percent catalyst. Preparations with catalyst concentrations of 0.04 and 0.023 wt. percent were made with a commercial hexane fraction as the water entrainer. Liquid temperatures were from  $100^{\circ}$ – $150^{\circ}$  C.

In the experiment with 0.023 wt. percent catalyst, a 25 mole percent excess of paraformaldehyde was added incrementally after the reaction between stoichiometric amounts had been completed.

The formal of  $C_{13}$  Oxo alcohol was prepared from the alcohol and paraformaldehyde with 2.4 wt. percent concentrated hydrochloric acid catalyst with a commercial hexane fraction as water entrainer at a final liquid temperature of  $131^{\circ}$  C. The flash of this product after distillation in a short path still at  $169^{\circ}$ – $176^{\circ}$  C. at 3 mm. was 370° F. but was raised to 405° F. by stripping at 80 microns with a rotating distillation column.

*Example 14*

The formal of  $C_{13}$  Oxo alcohol was prepared from the alcohol and paraformaldehyde in a stirred reactor by use of 0.2 wt. percent sodium acid sulfate catalyst and a commercial hexane fraction as a water entrainer at a liquid temperature of  $100^{\circ}$  C. Two moles of alcohol were treated with 0.75 mole of paraformaldehyde. After removal overhead of 11.5 ml. of water containing some formaldehyde, an additional 0.4 mole of paraformaldehyde was added and an additional 5.7 cc. of water entrained. The residue boiling above  $205^{\circ}$  C. at 20 mm. was taken as product.

*Example 15*

A pilot plant quantity of 131 lb. of the formal of  $C_{13}$  alcohol was prepared similarly to that in Example 15. A glass lined reactor was used and the yield on alcohol of the formal was 92 mol percent.

*Example 16*

The formal of  $C_{13}$  Oxo alcohol was prepared from  $C_{13}$  Oxo alcohol and paraformaldehyde using 0.1 wt. percent sodium acid sulfate with n-pentane as the water entrainer. The liquid temperature was  $100^{\circ}$  C. The residue boiling above  $165^{\circ}$  C. at 6 mm. was taken as product.

*Example 17*

The formal of  $C_{13}$  Oxo alcohol was prepared similarly to that in Example 17 except that the temperature of the liquid was  $90^{\circ}$  C. The residue boiling above  $163^{\circ}$  C. at 0.3 mm. was taken as product.

*Example 18*

The formal of  $C_{13}$  Oxo alcohol was prepared similarly to that in Example 17 except that the temperature of the liquid was  $90^{\circ}$  C. The residue boiling above  $163^{\circ}$  C. at 0.3 mm. was taken as product.

*Example 19*

The formal of  $C_{13}$  Oxo alcohol was prepared from the unchanged alcohol of Example 13. The entrainer was a commercial hexane fraction and the catalyst was 0.5

wt. percent sodium acid sulfate. The final liquid temperature was  $135^{\circ}$  C. The product distilled at  $167^{\circ}$ – $178^{\circ}$  C. at 5 mm.

*Example 20*

The formal of  $C_{13}$  Oxo alcohol was made by heating stoichiometric quantities of the alcohol and paraformaldehyde in a stainless steel bomb at  $100^{\circ}$  C. with 0.1, 0.5 and 2.5 wt. percent sodium acid sulfate catalyst. A similar experiment was run with 0.5 wt. percent p-toluenesulfonic acid catalyst. After heating in the bomb the water of reaction was separated mechanically and the reaction completed by entraining water with a commercial hexane fraction at a liquid temperature of below  $100^{\circ}$  C. The products were stripped of alcohol and the residue taken as the lubricant.

## Example 21

The formal of  $C_{13}$  Oxo alcohol was prepared by heating the alcohol with paraformaldehyde at  $100^\circ$  C. in the presence of 2.5 wt. percent sodium acid sulfate in a stirred flask fitted with a condenser. After stripping of alcohol the residue was taken as product.

## Example 22

The formal of  $C_{16}$  Oxo alcohol was made from the alcohol and paraformaldehyde with a commercial hexane fraction as entrainer and 1.2 wt. percent p-toluenesulfonic acid catalyst at a final liquid temperature of  $119^\circ$  C. The product distilled at  $206^\circ$ – $207^\circ$  C. at 7 mm.

## Example 23

The formal of 2-butyl-1-octanol was prepared by the method used in Example 22. It was taken as the residue boiling above  $175^\circ$  C. at 1.3 mm.

## Example 24

A formal of lauryl alcohol was prepared from the alcohol and aqueous formaldehyde solution by refluxing with 10 wt. percent concentrated hydrochloric acid catalyst. The residue boiling above  $205^\circ$  C. liquid temperature at 3 mm. was taken as product.

## Example 25

A  $C_{16}$  alcohol was prepared by the application of Guerbet's reaction to a  $C_8$  Oxo alcohol. A formal of this alcohol was made according to the procedure of Example 24 above.

Standard lubricant inspections were made on the products prepared as above and the results are set out in Table I below.

TABLE I

| Ex. No. | Formal of—                                   | Visc. in Cs. at— |         | Flash Point, °F. | ASTM Pour Point, °F. |
|---------|----------------------------------------------|------------------|---------|------------------|----------------------|
|         |                                              | 210° F.          | 100° F. |                  |                      |
| 1.      | $C_{10}$ Oxo Alcohol                         | 2.0              | 6.4     | 345              | -75                  |
| 2.      | $C_{11}$ Oxo Alcohol                         | 2.4              | 8.6     | 375              | -75                  |
| 3.      | Mixture of $C_{10}$ and $C_{13}$ Oxo alcohol | 2.61             | 9.91    | 370              | -75                  |
| 4.      | $C_{13}$ Oxo alcohol                         | 3.33             | 14.94   | 410              | <-75                 |
| 5.      | do                                           | 3.39             | 15.33   | 415              | -75                  |
| 10.     | do                                           |                  |         | 385              |                      |
| 12.     | do                                           | 3.41             | 15.23   | 370              | -75                  |
| 14.     | do                                           |                  |         | 370              |                      |
| 15.     | do                                           |                  |         | 405              |                      |
| 16.     | do                                           | 3.36             | 15.14   | 400              | -75                  |
| 17.     | do                                           |                  |         | 395              |                      |
| 18.     | do                                           |                  |         | 400              |                      |
| 19.     | do                                           | 3.32             | 15.1    | 380              | -75                  |
| 22.     | $C_{16}$ Oxo alcohol                         | 6.08             | 46.1    | 440              | -50                  |
| 23.     | 2-Butyl-1-Octanol                            | 2.30             | 8.65    | 385              | -75                  |
| 24.     | Lauryl alcohol                               | 3.22             | 10.63   | 400              | +65                  |
| 25.     | $C_{18}$ alcohol                             | 4.69             | 31.80   | 435              | -60                  |

It will be seen that all of the formals described in the table above are outstandingly useful as synthetic lubricants directly with the single exception that the formal of the straight chain alcohol of Example 24 has a high pour point. However, although the pour point of the formal of lauryl alcohol is too high to allow it to be used as a lubricating oil directly, it may be blended satisfactorily with other products.

These formals because of their extreme resistance to hydrolysis may be stripped with steam or distilled in the presence of water with or without an entraining agent present. Impurities such as unreacted formaldehyde may be removed by this method. Volatile catalysts used in the preparation of the formal also may be removed by this method and alkaline washing of the product thus avoided. Other materials which form azeotropes with water also may be removed from the formal by this method. Stripping with steam under vacuum may be used as the final purification step.

A further comparison of the formal of Example 4 was made with a mineral lubricating oil by subjecting a sample of each to the Lauson 25-hour engine test using a standard fuel. The engine was examined before and after the test and the merit ratings are given according to the test standards. Comparative data on this test using a formal of  $C_{13}$  Oxo alcohol and a highly refined mineral lubricating oil of 60 S. S. U. at  $210^\circ$  F.

TABLE II.—LAUSON ENGINE TEST  
[25 hours at  $300^\circ$  F.]

| 15 | Lubricant                           | Varnish Demerit <sup>1</sup> | Bearing Weight Loss (Gms./bearing) |
|----|-------------------------------------|------------------------------|------------------------------------|
|    | Mineral Oil.....                    | 4.75                         | 0.044                              |
|    | Formal of $C_{13}$ Oxo Alcohol..... | 2.25                         | 0.009                              |

<sup>1</sup> Rating scale 0 to 10; 0 being a perfect rating.

It is to be noted that the Lauson engine test data reported in Table II above point out that the varnish demerit rating for the formal of this invention is considerably better than that of the high quality lubricating oil and that the bearing weight loss is less than that experienced with the mineral oil. This indicates an overall advantage for the use of the synthetic lubricant of this invention.

## 30 FORMALS OF MONOETHERS OF POLYGLYCOLS

It has been found that a very satisfactory way of increasing the molecular weight of the formals of this invention is to add alkylene oxide units to an alcohol and then formalize two mols of the resulting product. The following examples set out preparations of various formals according to this concept.

In the examples below the formal usually was prepared as described under the formals of simple alcohols. This product was washed with an alkaline solution such as a saturated sodium carbonate or potassium carbonate solution or a carbonate-17% sodium chloride solution. After washing, the product was dried either by entrainment or over potassium carbonate and finally stripped at 1 to 10 mm. pressure.

## 45 Example 26

The mono-methyl ether of polypropylene glycol, prepared by adding propylene oxide to methanol in 9:1 mol ratio in the presence of sodium methoxide catalyst, followed by neutralization with 25% sulfuric acid to the sodium bisulfate stage, was converted to the formal by treatment with 66 mol percent excess paraformaldehyde in the presence of 1 wt. percent p-toluenesulfonic acid catalyst with a commercial hexane fraction as water entrainer. After washing with saturated potassium carbonate solution and stripping at 5 mm. to  $200^\circ$  C. liquid temperature, the residue was taken as product.

## Example 27

60 The mono-isopropyl ethers of two polypropylene glycols, prepared by adding propylene oxide to isopropyl alcohol in the presence of sodium isopropoxide catalyst, were converted to formals by treatment with paraformaldehyde in the presence of 1 wt. percent p-toluenesulfonic acid with a hexane fraction as a water entrainer. A stoichiometric amount of paraformaldehyde was used with the first example and a 100 mol percent excess in the second example.

65 Since the original mono-isopropyl ether of a polypropylene glycol may be used as a lubricant, the properties of the originals are compared with the properties of the formalized product below. It will be noted that the viscosity of the formal is higher but that the viscosity index is improved and that the pour is practically un-

75 changed.

| Lubricant                                                                                                          | Visc. in Cs. at— |         | Visc. Index | Flash Point, °F. | Pour Point, °F. |
|--------------------------------------------------------------------------------------------------------------------|------------------|---------|-------------|------------------|-----------------|
|                                                                                                                    | 210° F.          | 100° F. |             |                  |                 |
| IsoC <sub>8</sub> H <sub>7</sub> O(C <sub>2</sub> H <sub>5</sub> O) <sub>7.3</sub> *H                              | 4.32             | 20.6    | 136         | 415              | -65             |
| [IsoC <sub>8</sub> H <sub>7</sub> O(C <sub>2</sub> H <sub>5</sub> O) <sub>7.3</sub> ] <sub>2</sub> CH <sub>2</sub> | 7.35             | 35.8    | 154         | 390              | -60             |
| IsoC <sub>8</sub> H <sub>7</sub> O(C <sub>2</sub> H <sub>5</sub> O) <sub>8.6</sub> *H                              | 5.06             | 25.4    | 140         | 440              | -60             |
| [IsoC <sub>8</sub> H <sub>7</sub> O(C <sub>2</sub> H <sub>5</sub> O) <sub>8.6</sub> ] <sub>2</sub> CH <sub>2</sub> | 11.13            | 58.5    | 151         | 425              | -65             |

\*Calculated from the acetyl numbers.

It will be noted that the viscosity and viscosity index of the products of invention are quite outstanding as compared to the glycol monoethers.

#### Example 28

The mono-n-butyl ether of polypropylene glycol, prepared by reacting propylene oxide with n-butyl alcohol in the presence of sodium butoxide in a bomb, was converted to the formal by heating with a stoichiometric amount of paraformaldehyde in the presence of a hexane fraction as entrainer with 1 wt. percent p-toluenesulfonic acid as a catalyst. The mono-ether of the glycol is compared with its formal in order to show the improvement in viscosity and viscosity index. The pour remains excellent.

| Lubricant                                                                                                       | Visc. in Cs. at— |         | Visc. Index | Flash Point, °F. | Pour Point, °F. |
|-----------------------------------------------------------------------------------------------------------------|------------------|---------|-------------|------------------|-----------------|
|                                                                                                                 | 210° F.          | 100° F. |             |                  |                 |
| C <sub>4</sub> H <sub>9</sub> O(C <sub>2</sub> H <sub>5</sub> O) <sub>7.4</sub> H                               | 4.38             | 21.3    | 133         | 400              | <-75            |
| [C <sub>4</sub> H <sub>9</sub> O(C <sub>2</sub> H <sub>5</sub> O) <sub>7.4</sub> ] <sub>2</sub> CH <sub>2</sub> | 6.50             | 31.5    | 154         | 400              | -70             |

#### Example 29

The mono-n-butyl ether of polypropylene glycol, prepared by adding propylene oxide to n-butyl alcohol in a 7:1 mol ratio in the presence of sodium butoxide catalyst at atmospheric pressure, was converted to the formal by heating with 72 mol percent excess paraformaldehyde in the presence of 1 wt. percent p-toluenesulfonic acid catalyst with a heptane fraction as water entrainer. The product was washed, dried over anhydrous potassium carbonate and topped to a 200° C. liquid temperature at 3 mm.

| Lubricant                                                                           | Visc. in Cs. at— |         | Visc. Index | Flash Point, °F. | Pour Point, °F. |
|-------------------------------------------------------------------------------------|------------------|---------|-------------|------------------|-----------------|
|                                                                                     | 210° F.          | 100° F. |             |                  |                 |
| [n-BuO(C <sub>2</sub> H <sub>5</sub> O) <sub>7</sub> ] <sub>2</sub> CH <sub>2</sub> | 6.30             | 28.8    | 153         | 405              | -65             |

Formals of similar products were made using sodium acid sulfate catalyst at 1 wt. percent concentration and a C<sub>6</sub> as well as a C<sub>7</sub> hydrocarbon fraction as entrainer.

#### Example 30

A commercial mono-n-butyl ether of polypropylene glycol of approximately 1000 mol wt. was treated with a stoichiometric amount of paraformaldehyde in the presence of 1 wt. percent sodium acid sulfate catalyst and a C<sub>7</sub> hydrocarbon fraction as entrainer. The improvement in viscosity and retention of an excellent viscosity index and pour point as a result of conversion to the formal is shown below.

| Lubricant                                                                                                      | Visc. in Cs. at— |         | Visc. Index | Flash Point, °F. | Pour Point, °F. |
|----------------------------------------------------------------------------------------------------------------|------------------|---------|-------------|------------------|-----------------|
|                                                                                                                | 210° F.          | 100° F. |             |                  |                 |
| C <sub>4</sub> H <sub>9</sub> O(C <sub>2</sub> H <sub>5</sub> O) <sub>16</sub> H                               | 14.4             | 85.2    | 143         | 440              | -45             |
| [C <sub>4</sub> H <sub>9</sub> O(C <sub>2</sub> H <sub>5</sub> O) <sub>16</sub> ] <sub>2</sub> CH <sub>2</sub> | 21.4             | 127.5   | 143         | 430              | -45             |

#### Example 31

The mono-isoctyl ethers of four polyethylene glycols, prepared from C<sub>8</sub> Oxo alcohol and ethylene oxide with boron fluoride catalyst, were treated with stoichiometric amounts of paraformaldehyde with 1 wt. percent sodium acid sulfate catalyst and a C<sub>7</sub> hydrocarbon fraction as the water entrainer. The formal of C<sub>8</sub>H<sub>17</sub>O(C<sub>2</sub>H<sub>5</sub>O)<sub>8.6</sub>H also was prepared using 1 wt. percent p-toluenesulfonic acid catalyst. The properties of these formals are given below. The pour points and viscosity indices are exceptionally good.

| Lubricant                                                                                                          | Visc. in Cs. at— |         | Visc. Index | Flash Point, °F. | Pour Point, °F. |
|--------------------------------------------------------------------------------------------------------------------|------------------|---------|-------------|------------------|-----------------|
|                                                                                                                    | 210° F.          | 100° F. |             |                  |                 |
| IsoC <sub>8</sub> H <sub>17</sub> O(C <sub>2</sub> H <sub>5</sub> O) <sub>3.1</sub> ] <sub>2</sub> CH <sub>2</sub> | 3.97             | 15.0    | 186         | 400              | <-75            |
| IsoC <sub>8</sub> H <sub>17</sub> O(C <sub>2</sub> H <sub>5</sub> O) <sub>4.7</sub> ] <sub>2</sub> CH <sub>2</sub> | 5.08             | 21.5    | 170         | 400              | <-75            |
| IsoC <sub>8</sub> H <sub>17</sub> O(C <sub>2</sub> H <sub>5</sub> O) <sub>6.3</sub> ] <sub>2</sub> CH <sub>2</sub> | 6.12             | 22.3    | 166         | 410              | -50             |
| IsoC <sub>8</sub> H <sub>17</sub> O(C <sub>2</sub> H <sub>5</sub> O) <sub>8.6</sub> ] <sub>2</sub> CH <sub>2</sub> | 5.74             | 26.0    | 161         | 420              | -30             |
| IsoC <sub>8</sub> H <sub>17</sub> O(C <sub>2</sub> H <sub>5</sub> O) <sub>8.6</sub> ] <sub>2</sub> CH <sub>2</sub> | 7.26             | 32.7    | 162         | 420              | -35             |

\* Prepared with sodium acid sulfate.

† Prepared with p-toluenesulfonic acid.

#### Example 32

The mono-isoctyl ethers of four polypropylene glycols were prepared from C<sub>8</sub> Oxo alcohol and propylene oxide with sodium iso-octoxide catalyst. These were converted to the formals by reaction with paraformaldehyde using 1 wt. percent p-toluenesulfonic acid catalyst and a C<sub>6</sub> hydrocarbon fraction as a water entrainer. The first example was treated twice with stoichiometric amounts of paraformaldehyde, the second, twice with stoichiometric amounts and once with half of a stoichiometric amount. In the last two examples, the alcohol was treated once with a stoichiometric amount of paraformaldehyde. The properties of the glycols and the corresponding formals are shown in the table below. In every case an increase in viscosity resulted while the viscosity index increased and the pour point remained excellent.

| Lubricant                                                                                                          | Visc. in Cs. at— |         | Visc. Index | Flash Point, °F. | Pour Point, °F. |
|--------------------------------------------------------------------------------------------------------------------|------------------|---------|-------------|------------------|-----------------|
|                                                                                                                    | 210° F.          | 100° F. |             |                  |                 |
| IsoC <sub>8</sub> H <sub>17</sub> O(C <sub>2</sub> H <sub>5</sub> O) <sub>4.1</sub> H                              | 2.55             | 11.0    | 52          | 310              | <-75            |
| IsoC <sub>8</sub> H <sub>17</sub> O(C <sub>2</sub> H <sub>5</sub> O) <sub>4.1</sub> ] <sub>2</sub> CH <sub>2</sub> | 4.97             | 22.2    | 162         | 400              | <-75            |
| IsoC <sub>8</sub> H <sub>17</sub> O(C <sub>2</sub> H <sub>5</sub> O) <sub>5.8</sub> H                              | 3.04             | 13.7    | 80          | 370              | <-75            |
| IsoC <sub>8</sub> H <sub>17</sub> O(C <sub>2</sub> H <sub>5</sub> O) <sub>5.8</sub> ] <sub>2</sub> CH <sub>2</sub> | 6.65             | 31.5    | 158         | 410              | <-75            |
| IsoC <sub>8</sub> H <sub>17</sub> O(C <sub>2</sub> H <sub>5</sub> O) <sub>7.0</sub> H                              | 4.25             | 21.3    | 130         | 400              | <-75            |
| IsoC <sub>8</sub> H <sub>17</sub> O(C <sub>2</sub> H <sub>5</sub> O) <sub>7.0</sub> ] <sub>2</sub> CH <sub>2</sub> | 7.11             | 35.4    | 152         | 405              | -60             |
| IsoC <sub>8</sub> H <sub>17</sub> O(C <sub>2</sub> H <sub>5</sub> O) <sub>8.6</sub> H                              | 5.22             | 26.8    | 138         | 415              | <-75            |
| IsoC <sub>8</sub> H <sub>17</sub> O(C <sub>2</sub> H <sub>5</sub> O) <sub>8.6</sub> ] <sub>2</sub> CH <sub>2</sub> | 8.59             | 44.7    | 150         | 420              | -55             |

#### Example 33

The mono-isodecyl ethers of ethylene glycol and of diethylene glycol were prepared from C<sub>10</sub> Oxo alcohol and ethylene oxide with boron fluoride catalyst. They were converted to formals by their reaction with stoichiometric amounts of paraformaldehyde in the presence of 1 wt. percent sodium acid sulfate catalyst, with a C<sub>6</sub> hydrocarbon as the entrainer in the first example and a C<sub>7</sub> hydrocarbon as the entrainer in the second example. The properties of these formals which were distilled under reduced pressure are as follows:

| Lubricant                                                                           | Visc. in Cs. at— |         | Visc. Index | Flash Point, °F. | Pour Point, °F. |
|-------------------------------------------------------------------------------------|------------------|---------|-------------|------------------|-----------------|
|                                                                                     | 210° F.          | 100° F. |             |                  |                 |
| $[\text{IsoC}_{10}\text{H}_{21}\text{O}(\text{O}_2\text{H}_4\text{O})_2\text{CH}_2$ | 2.64             | 9.24    | 136         | 360              | $<-75$          |
| $[\text{IsoC}_{10}\text{H}_{21}\text{O}(\text{O}_2\text{H}_4\text{O})_2\text{CH}_2$ | 3.71             | 14.08   | 173         | 390              | $<-75$          |

A mono-isodecyl ether of diethylene glycol was prepared by the addition of ethylene oxide to  $\text{C}_{10}$  Oxo alcohol in a mol ratio of 2:1 with boron fluoride catalyst. The product was not isolated. To this synthesis mixture was added a stoichiometric amount of paraformaldehyde, 1 wt. percent of sodium acid sulfate and a  $\text{C}_7$  hydrocarbon fraction as an entrainer. After the reaction was completed, the mixture was washed with alkali and topped to a liquid temperature of 210° F. at 1 mm. The formal of the monoisodecyl ether of tetraethylene glycol was similarly prepared and topped to a liquid temperature of 234° C. at 1 mm. This last compound was also prepared with 2.5 wt. percent p-toluenesulfonic acid as the formalization catalyst both with an entrainer and in a bomb. The results were good.

| Lubricant                                                                           | Visc. in Cs. at— |         | Visc. Index | Flash Point, °F. | Pour Point, °F. |
|-------------------------------------------------------------------------------------|------------------|---------|-------------|------------------|-----------------|
|                                                                                     | 210° F.          | 100° F. |             |                  |                 |
| $[\text{C}_{10}\text{H}_{21}\text{O}(\text{C}_2\text{H}_4\text{O})_2]_2\text{CH}_2$ | 4.72             | 19.57   | 180         | 425              | $<-75$          |
| $[\text{C}_{10}\text{H}_{21}\text{O}(\text{C}_2\text{H}_4\text{O})_4]_2\text{CH}_2$ | 6.40             | 28.2    | 166         | 460              | -40             |

#### Example 34

The mono-isotridecyl ether of ethylene glycol, prepared from  $\text{C}_{13}$  Oxo alcohol and ethylene oxide with boron fluoride catalyst, was converted to its formal by treatment with a stoichiometric amount of paraformaldehyde in the presence of 1 wt. percent sodium acid sulfate catalyst and a  $\text{C}_7$  hydrocarbon fraction as the water entrainer. Similar preparations were made of formals of  $\text{C}_{13}$  ethers of polyethylene glycols which correspond closely to formulas for penta- and octa-ethylene glycols. The properties are as follows:

| Lubricant                                                                              | Visc. in Cs. at— |         | Visc. Index | Flash Point, °F. | Pour Point, °F. |
|----------------------------------------------------------------------------------------|------------------|---------|-------------|------------------|-----------------|
|                                                                                        | 210° F.          | 100° F. |             |                  |                 |
| $[\text{IsoC}_{13}\text{H}_{27}\text{O}(\text{C}_2\text{H}_4\text{O})_2]_2\text{CH}_2$ | 2.55             | 15.0    | 96          | 275              | $<-75$          |
| $[\text{IsoC}_{13}\text{H}_{27}\text{O}(\text{C}_2\text{H}_4\text{O})_4]_2\text{CH}_2$ | 6.55             | 34.6    | 145         | 440              | -70             |

In the examples given above both A and B of the formula  $\text{A}-\text{O}-\text{CH}_2-\text{O}-\text{B}$  are represented by a glycol monoether, that is to say, the formal has the structure

Glycol monoether—formal—glycol monoether

The invention also contemplates materials wherein A is a glycol monoether and B is an alcohol. These can be represented by the formula



wherein R is a hydrocarbon group, n is a number from 2 to 5 and x is a number from 1 to 50.

The following example illustrates this concept.

#### Example 35

The hemiformal of  $\text{C}_8$  Oxo alcohol was prepared by heating 130 g. (1 mole) of the alcohol with 30.1 g. (1 mole  $\text{CH}_2\text{O}$ ) trioxymethylene, 200 g. heptane and 10 g.  $\text{NaHSO}_4$  catalyst for 25 minutes (until the formaldehyde dissolves) at 65° C. To this hemiformal was then added

75 Example 39 below.

887 g. (1 mole) of deca-propylene glycol mono-n-butyl ether and 100 g. heptane. The mixture was then refluxed at 100° to 117° C. over a period of 100 minutes during which time 20.8 cc. of water was collected. A fine muddy precipitate formed early in the reaction. This was filtered off along with the catalyst. After stripping, the material had the following properties:

| 10 | Visc. in Cs. at— |         | Visc. Index | Flash Point, °F. | Pour Point, °F. |
|----|------------------|---------|-------------|------------------|-----------------|
|    | 210° F.          | 100° F. |             |                  |                 |
|    | 7.72             | 39.68   | 150         | 420              | -65             |

#### FORMALS OF HYDROXY ACID ESTERS

Esters of hydroxy acids may also be used to prepare valuable materials.

##### Example 36

Alpha-hydroxydecanoic acid was esterified with an equivalent quantity of  $\text{C}_8$  Oxo alcohol with 1 wt. percent p-toluenesulfonic acid as a catalyst and a  $\text{C}_6$  hydrocarbon fraction as a water entrainer. At the end of the esterification a stoichiometric amount of paraformaldehyde was added and the theoretical amount of water entrained at a maximum liquid temperature of 109° C. After washing and distillation at 160°–180° C. at 1.5 mm. pressure the product gave a saponification value of 99.7% of the theoretical.

The lubricant inspections on this product were as follows:

| 35 | Lubricant                                  | Visc. in Cs. at— |         | Flash Point, °F. | Pour Point, °F. |
|----|--------------------------------------------|------------------|---------|------------------|-----------------|
|    |                                            | 210° F.          | 100° F. |                  |                 |
|    | Formal of Isooctyl-alpha-hydroxy decanoate | 6.74             | 65.3    | 385              | -25             |

##### Example 37

Lactic acid, 85% in water, was esterified with an equivalent amount of  $\text{C}_{13}$  Oxo alcohol in the presence of 1 wt. percent sodium acid sulfate as catalyst with a  $\text{C}_7$  hydrocarbon fraction as an entrainer. After removal of the water of esterification plus the water of the lactic acid solution, an equivalent amount of paraformaldehyde was added and the theoretical amount of water removed at a maximum liquid temperature of 128° C. After washing, the distillate boiling at 205°–240° C. at 1 mm. was taken as product.

The lubricant inspections on this product were as follows:

| 55 | Lubricant                     | Visc. in Cs. at— |         | Flash Point, °F. | Pour Point, °F. |
|----|-------------------------------|------------------|---------|------------------|-----------------|
|    |                               | 210° F.          | 100° F. |                  |                 |
|    | Formal of Isotridecyl lactate | 3.32             | 15.36   | 400              | -70             |

##### Example 38

The formal of isodecyl lactate was made by the procedure given in Example 37. It distilled at 160°–195° C. at 2 mm.

| 60 | Lubricant                  | Visc. in Cs. at— |         | Flash Point, °F. | Pour Point, °F. |
|----|----------------------------|------------------|---------|------------------|-----------------|
|    |                            | 210° F.          | 100° F. |                  |                 |
|    | Formal of Isodecyl lactate | 3.32             | 15.36   | 400              | -70             |

##### Example 38

Formals of glycol monoesters may also be prepared and have excellent lubricity characteristics as is shown by Example 39 below.

## 15

## Example 39

The monoester of dipropylene glycol and pelargonic acid was first made by heating 268.3 g. (2 moles) of dipropylene glycol with 303 g. (2 moles) of pelargonic acid, 100 g. heptane and 5.7 g. NaHSO<sub>4</sub> catalyst. Esterification time was 2.25 hours during which time the temperature increased from 107° C. to 124° C. and the volume of water collected was 37.2 cc. (theoretical is 36 cc.). The reaction mixture was then allowed to cool. One mole (30 g.) of paraformaldehyde and 100 cc. of heptane were added and the mixture heated to a reflux temperature of 101° C. After one hour the temperature had increased to 115° C. and 18.0 cc. of water had collected. On continued heating no more water was evolved. The reaction mixture was washed with three 100 cc. portions of 10% Na<sub>2</sub>CO<sub>3</sub> solution and then three 100 cc. portions of water. The reaction mixture was stripped free of heptane and light ends. The material boiling above 145° C. at 0.4 mm. (kettle temperature of 180° C.) had the following properties:

| Visc. in Cs. at— |         | Flash Point,<br>°F. | Pour Point,<br>°F. |
|------------------|---------|---------------------|--------------------|
| 210° F.          | 100° F. |                     |                    |
| 3.06             | 11.75   | 390                 | <-75               |

The material boiling above 185° C. at 0.11 mm. (kettle temperature of 211° C.) and constituting the glycol monoester formal of this invention had the following properties:

| Visc. in Cs. at— |         | Pour Point,<br>°F. |
|------------------|---------|--------------------|
| 210° F.          | 100° F. |                    |
| 4.36             | 19.66   | <-75               |

It will be seen that the formals of this invention have viscosity characteristics at both low and high temperatures that make them especially desirable as synthetic lubricants. It will be noted that all of the materials listed in the tables have flash points that are in excess of 350° F. and viscosities at 210° F. and 100° F. which are well within the limitations essential to synthetic lubricating compositions.

## GREASES

It has also been found that lubricating compositions prepared by thickening the formals of this invention, or blends of these formals with other synthetic lubricants or with mineral oils, with grease forming soaps have desirable properties which make them especially advantageous for the lubrication of moving metal parts where a liquid cannot be used. These grease compositions are simply and economically prepared using as a thickening agent any of the common grease forming soaps. The alkali or alkaline earth metal soaps of high molecular weight substantially saturated fatty acids are used and the grease compositions prepared by any of the methods with which the art is familiar. For instance, soaps such as the oleates, stearates or ricinoleates of sodium, potassium, lithium, calcium, barium, strontium, aluminum, iron, zinc, copper and the like may be used as thickeners for the formals of the invention as well as soaps formed by heating animal, fish, or vegetable oils with soda, lime, baria hydrate or lithia hydrate. Examples of some of these grease compositions are set out below.

## 16

## Example 40

## FORMULATION

- 5 7.5% lithium stearate  
7.5% lithium hydroxy stearate  
0.5% phenothiazine  
84.5% formal of C<sub>10</sub> Oxo alcohol

## PREPARATION

10 The combined soaps were dispersed cold in the formal and heated while stirring to 400° F. At this temperature the inhibitor (phenothiazine) was added and the mass poured into a shallow pan for cooling. When cold the grease was homogenized to a soft uniform consistency.

## PROPERTIES

- 20 Appearance..... Light cream color, smooth, buttery.  
Penetrations, 77° F., mm./10:  
Unworked..... 280.  
Worked (60 strokes)..... 300.  
Worked (100,000 strokes)..... 360.  
25 Dropping point (° F.)..... 365.  
Water solubility..... Nil (boiling water).  
Norma Hoffman oxidation test  
(hours to 5 p. s. i. drop in oxygen pressure)..... 291.

## Example 41

## FORMULATION

- 35 7.5% lithium stearate  
7.5% lithium hydroxy stearate  
0.5% phenothiazine  
84.5% formal of C<sub>13</sub> Oxo alcohol

## PREPARATION

40 Same as Example 40.

## PROPERTIES

- 45 Appearance..... Light cream color, smooth, buttery.  
Penetrations, 77° F., mm./10:  
Unworked..... 275.  
Worked (60 strokes)..... 295.  
Worked (100,000 strokes)..... 340.  
50 Dropping point (° F.)..... 365.  
Water solubility..... Nil (boiling water).  
Norma Hoffman oxidation test  
(hours to 3 p. s. i. drop in oxygen pressure)..... 200.

## Example 42

## FORMULATION

- 60 7.5% lithium stearate  
7.5% lithium hydroxy stearate  
20.0% formal of C<sub>10</sub> Oxo alcohol  
64.0% complex ester (adipic acid-C<sub>8</sub> Oxo alcohol-1-3 butanediol)  
65 1.0% phenyl-alpha-naphthylamine

## PREPARATION

70 The combined soaps were mixed with the formal and heated to 350° F. At this temperature the soap began to swell and disperse in the formal. The complex ester was then slowly added while continuing to stir and heat and the mass heated to 400° F. until all the soap was in solution. Phenyl-alpha-naphthylamine inhibitor was added and the grease cooled in shallow pans.

17  
PROPERTIES

|                                                                               |                                                   |
|-------------------------------------------------------------------------------|---------------------------------------------------|
| Appearance                                                                    | Light brown, slightly rough texture, short fiber. |
| Penetrations, 77° F., mm./10:                                                 |                                                   |
| Unworked                                                                      | 280.                                              |
| Worked (60 strokes)                                                           | 285.                                              |
| Worked (100,000 strokes)                                                      | 340.                                              |
| Dropping point (° F.)                                                         | 370.                                              |
| Norma Hoffman oxidation test<br>(hours to 5 p. s. i. drop in oxygen pressure) | 332.                                              |

## Example 43

## FORMULATION

20.0% lithium fatty acid soaps (Litholite)  
1.0% phenyl alpha-naphthylamine  
79.0% mixed formal of decapropylene glycol mono-n-butyl ether and C<sub>8</sub> Oxo alcohol, e. g.  
n-C<sub>4</sub>H<sub>9</sub>O(C<sub>3</sub>H<sub>6</sub>O)<sub>10</sub>—CH<sub>2</sub>—O—iso—C<sub>8</sub>H<sub>17</sub>

## PREPARATION

The soap was dispersed in the synthetic lubricant by heating to 400° F. with stirring. After the soap dissolved the phenyl alpha-naphthylamine was added and the mixture was pan cooled. An excellent light brown color grease having a good grease structure was obtained. The dropping point of the grease was 364° F.

## DETERGENT BLENDS

In the manufacture of detergent additives for mineral lubricating oils, it has been found necessary in some instances to use agents to solubilize or plasticize the additives before blending into a mineral oil, either to prepare a concentrate or to prepare the finished oil blend. In the past materials such as stearyl alcohol, coconut oil alcohols, or other long chain alcoholic materials having been used. However, for use with detergent materials such as salts of alkylated phenols and their derivatives, such as the sulfurized barium salt of tert.-octyl phenol and the reaction product of such material with a phosphorus sulfide, such as P<sub>2</sub>S<sub>5</sub>, these alcohols are not entirely satisfactory since they may prevent a rapid filtration rate on the final blend. It has been found, however, that formals prepared in accordance with the concept of this invention are very satisfactory for use as solubilizers or plasticizers for the alkylated phenol type additive. As an example, a sample of a sulfurized barium salt of tert.-octyl phenol and a sample of the P<sub>2</sub>S<sub>5</sub>-treated sulfurized barium salt of tert.-octyl phenol was prepared with 5% of stearyl alcohol and with 5% of the formal of C<sub>8</sub> Oxo alcohol. These four samples were submitted for analysis of barium, sulfur, and phosphorus content, viscosity at 210° F., a color test, and a copper strip test.

The color was measured on the standardized commercial TAG-Robinson Colorimeter, by which lighter colors have higher numbers, the corrosion of copper strip was measured by ASTM procedure D-130 with a semi-quantitative scale of measurements wherein 8 and 10 is very bad, 5 and 7 is acceptable, 2 and 4 is very good and 1 is perfect.

The results of these tests are set out below, and show the advantage of the formal over the stearyl alcohol as a plasticizer.

|                        | Detergent A            | Detergent B            | Detergent A               | Detergent B               |
|------------------------|------------------------|------------------------|---------------------------|---------------------------|
| Plasticizer (5%)       | C <sub>18</sub> alcoh. | C <sub>18</sub> alcoh. | C <sub>8</sub> Oxo formal | C <sub>8</sub> Oxo formal |
| Percent Barium         | 8.89                   | 8.14                   | 8.67                      | 8.54                      |
| Percent Sulfur         | 3.09                   | 5.79                   | 3.08                      | 5.42                      |
| Percent Phosphorus     | 10.25                  | 9.86                   | 10.25                     | 10.91                     |
| Color                  | 3                      | 7                      | 3                         | 6                         |
| Copper Strip Test      | 142                    | 169.8                  | 122.4                     | 159.4                     |
| Visc. at 210° F. (SUS) |                        |                        |                           |                           |

A = Barium salt of tert.-octyl phenol sulfide.

B = Detergent A treated with P<sub>2</sub>S<sub>5</sub>.

18  
VISCOSITY INDEX IMPROVER BLENDS

Another interesting feature in connection with addition agents for use with the materials of this invention arises in respect to the addition of thickening agents. The 5 formal prepared by joining two molecules of C<sub>13</sub> Oxo alcohol has a viscosity at 210° F. of 37 SUS, which is lower than is considered optimum. It has been found that this formal may be thickened to a level of about 49 SUS at 210° F. by inclusion of either 2.45 wt. percent of a low molecular weight polybutene (16,400 m. wt.) or about 11.8 wt. percent of a 25% mineral oil solution of the same. This thickening with an olefinic polymer is somewhat unusual because hydrocarbon high polymers have hitherto been found incompatible with oxy-type 15 polymeric synthetic lubricants, showing phase separation at room temperature. The reason for the unusual behavior is believed to be associated with the carbon to oxygen ratio. In most synthetic lubricants, especially diesters and complex esters, the carbon to oxygen ratio will be between about 4:1 to 7:1. In the C<sub>13</sub> Oxo formal this ratio is 13.5:1. This is two or three times higher than for the best diesters and complex esters. Consequently, it may be postulated that the solubility characteristics of the C<sub>13</sub> Oxo formal approach those of a hydrocarbon or mineral oil. The effect of the ether oxygen in the C<sub>13</sub> Oxo formal is not entirely submerged, since only about 10 wt. percent of the polybutene will dissolve therein, whereas the solubility of the formal in mineral 20 oils appears to be unlimited.

It would appear, therefore, that for satisfactory thickening of ether-oxygen containing polymers with the polybutene type of thickening agents, the lubricant must have a carbon to oxygen ratio falling within the range of about 7:1 to 50:1.

One method of adding the thickener, of course, is to add the solid polymer and heat and stir to dissolve. Another method is to dissolve the polymer in hexane or some other hydrocarbon solvent and remove the solvent by stripping. Still another method is to add the thickener 40 in a hydrocarbon solution to the crude formal lubricant either before or after it is washed free of acid catalyst. In the latter method any unchanged alcohol and hydrocarbon entrained is removed in the same operation as the hydrocarbon solvent for the thickener. The advantages are ease of handling of the thickener and also removal 45 of any light hydrocarbon materials that may be present in the supposedly pure thickener.

Polymers and copolymers of acrylic and methacrylic acid esters may also be used to improve the viscosity 50 index of the formals of invention. Other well known viscosity index improvers such as copolymers of esters of dibasic acids and vinyl compounds may also be used.

As has been mentioned, the formals of this invention 55 may be improved by the use of many different types of additive agents. The great thermal stability of the formals and their resistance to oxidation in the presence of inhibitors makes possible their use in many different processes as heat transfer liquids. These stabilized materials, exemplified by a bis-C<sub>13</sub> Oxo formal fortified by small amounts of such antioxidants as phenyl alpha-naphthylamine, phenothiazine, 2,6-di-tert.-butyl-para- cresol, etc. may be used as heat transfer agents at temperatures up to about 500° F.

To summarize, this invention relates to new compositions of matter which have outstanding utility as synthetic 60 lubricating oils. The materials of this invention may be broadly described as being the formals of organic materials containing at least one hydroxyl group that is alcoholic in nature. The structure of the formals of invention may be described as being one corresponding to the formula:



wherein A and B are organic radicals containing from 1 to 60 carbon atoms and are derived from the organic 75 materials containing the alcoholic hydroxyl group. A

and B may be alike or different, and the total number of carbon atoms in the molecule should be between 20 and 130, preferably between 25 and 100. The compounds that are especially preferred are those materials that have a kinematic viscosity at 210° F. within the range of 2 to 60 centistokes, an ASTM pour point of at least as low as 35° F., and a flash point of at least 300° F. The formals of this invention are suitable as plasticizers, solubilizers, heat transfer agents, grease bases, insecticides, weed killers, rust preventatives, solvents, as for gum in gasoline, dewaxing aids, detergents, oiliness agents as in penetrating oils, and as raw materials for many other industrial applications. These new compositions may be admixed with mineral oils either as concentrates or as finished blends. They may be blended with other synthetic lubricants such as dibasic acid esters, complex esters, polymerized hydrocarbons and the like. They are compatible to the addition of well-known additive agents and finished blends may contain viscosity index improvers, pour point depressants, detergents, antioxidants, rust inhibitors, and the like.

The instant application is a continuation-in-part of application Serial No. 288,301, filed May 16, 1952, now Patent No. 2,746,924.

What is claimed is:

1. As a synthetic lubricant, a formal having an ASTM pour point below about 35° F., a flash point above about 300° F., and a kinematic viscosity at 210° F. within the range of 2 to 60 centistokes, said formal having the formula



wherein A contains 1 to 60 carbon atoms and is selected from the group consisting of hydrocarbon and substituted hydrocarbon radicals, and B contains 1 to 60 carbon atoms and is selected from the group consisting of hydrocarbon radicals containing ether linkages and hydrocarbon radicals containing ester linkages, said formal containing at least 20 carbon atoms per molecule.

2. As a synthetic lubricant, a formal having an ASTM pour point below about 35° F., a flash point above about 300° F., and a kinematic viscosity at 210° F. within the range of 2 to 60 centistokes, said formal having the formula



wherein A and B contain from 1 to 60 carbon atoms and are selected from the group consisting of hydrocarbon radicals containing ether linkages and hydrocarbon radicals containing ester linkages, said formal containing at least 20 carbon atoms per molecule.

3. As a synthetic lubricant, a formal having an ASTM pour point below about 35° F., a flash point above about 300° F., and a kinematic viscosity at 210° F. within the

range of 2 to 60 centistokes, said formal being selected from the group consisting of formals of glycol monoether and formals of glycol monoester, and containing about 20 to 130 carbon atoms in the molecule.

4. As a synthetic lubricant a formal having an ASTM pour point below about 35° F., a flash point above about 300° F., and a kinematic viscosity at 210° F. within the range of 2 to 60 centistokes, said formal having the formula



wherein R is an alkyl group of from 1 to 20 carbon atoms and wherein n and x are numbers greater than zero, said formal containing about 20 to 130 carbon atoms per molecule.

5. As a synthetic lubricant, a formal having a pour point below about 35° F., a flash point above about 300° F., and a kinematic viscosity at 210° F. within the range of 2 to 60 centistokes, said formal having the formula



wherein R is an alkyl group of from 1 to 20 carbon atoms and wherein n and x are numbers greater than zero, said formal containing a total of about 20 to 130 carbon atoms per molecule.

6. As a synthetic lubricant, a formal having an ASTM pour point below about 35° F., a flash point above about 300° F., and a kinematic viscosity at 210° F. within the range of 2 to 60 centistokes, said formal being formed from an ester of a hydroxy acid and containing a total of about 20 to 130 carbon atoms per molecule.

#### References Cited in the file of this patent

#### UNITED STATES PATENTS

|    |           |               |       |               |
|----|-----------|---------------|-------|---------------|
| 35 | 2,036,304 | Seymour       | ----- | Apr. 7, 1936  |
|    | 2,321,557 | Sussman       | ----- | June 8, 1943  |
|    | 2,350,350 | Gresham       | ----- | June 6, 1944  |
|    | 2,379,703 | Geltner       | ----- | July 3, 1945  |
|    | 2,388,409 | Harvey        | ----- | Nov. 6, 1945  |
|    | 2,397,602 | Gresham       | ----- | Apr. 2, 1946  |
|    | 2,436,347 | Zimmer et al. | ----- | Feb. 17, 1948 |
|    | 2,473,994 | Gresham       | ----- | June 21, 1949 |
| 30 | 2,512,722 | Lanham        | ----- | July 27, 1950 |
|    | 2,585,182 | Sterman       | ----- | Feb. 12, 1952 |
|    | 2,628,974 | Sanderson     | ----- | Feb. 17, 1953 |

#### FOREIGN PATENTS

|    |         |               |       |               |
|----|---------|---------------|-------|---------------|
| 40 | 425,396 | Great Britain | ----- | Mar. 13, 1935 |
|    | 879,689 | France        | ----- | Nov. 30, 1942 |

#### OTHER REFERENCES

Kursanov et al.: Abstracted in Chem. Abs. 42, page 4922 (1948).